

No. 746,796.

PATENTED DEC. 15, 1903.

P. DANCKWARDT.

PROCESS OF SIMULTANEOUSLY PRODUCING ALKALI CYANID AND  
ALKALI METAL.

APPLICATION FILED JUNE 10, 1903.

NO MODEL.

FIG. 1



FIG. 2



Witnesses:

Arthur J. Jeppe.  
Edward Ray.

Inventor:

Paul Danckwardt  
by his attorney  
Paul M. Biresaw

## UNITED STATES PATENT OFFICE.

PAUL DANCKWARDT, OF DEADWOOD, SOUTH DAKOTA.

## PROCESS OF SIMULTANEOUSLY PRODUCING ALKALI CYANID AND ALKALI METAL.

SPECIFICATION forming part of Letters Patent No. 746,796, dated December 15, 1903.

Application filed June 10, 1903. Serial No. 160,866. (No specimens.)

*To all whom it may concern:*

Be it known that I, PAUL DANCKWARDT, a citizen of the United States, residing at Deadwood, Lawrence county, South Dakota, have 5 invented certain new and useful Improvements in Processes of Simultaneously Producing Alkali Cyanid and Alkali Metal, of which the following is a specification.

This invention relates to a process of producing simultaneously an alkali cyanid and an alkali metal; and it consists in heating a mixture of the nitrite of an alkali metal with another salt of an alkali metal and the carbid of an alkali-earth metal under exclusion of air. As a nitrite I prefer sodium nitrite, ( $NaNO_2$ ) and as a carbid the carbid of calcium, ( $CaC_2$ ). The other alkali salt may be any salt that does not contain oxygen, as that would require a larger amount of the 15 reducing agent or would otherwise create an oxidizing effect on the end products, alkali cyanid and alkali metal.

In the accompanying drawings, Figure 1 is a vertical section of a furnace for carrying 20 my process into effect on line 11, Fig. 2; and Fig. 2 is a horizontal section on line 2 2, Fig. 1.

The furnace consists of a box the sides of 25 which are formed by four water-jackets *a*, resting on a basic foundation *b* and connected by braces *c*. One of the jackets has an opening or tap-hole *a'*, with a sprout *d*. Two opposite jackets *a* have openings through which the insulated carbon resistance-blocks *e* are 30 introduced. These blocks carry on their outer ends clamps *e'* for connection with the poles of a dynamo. The box is provided with a cover *f*, having a charging-manhole which is closed by a lid *f'*. A pipe *g* conveys the 35 gasic metal to a closed receptacle *h*.

In order to carry the process into effect by the above-described apparatus, I fill the box with the mixed ingredients in about the following proportions, by weight: one hundred 40 and thirty-eight parts of sodium nitrite, one hundred and ninety-five parts of fluorid of sodium, two hundred and fifty-five parts 45 of carbid of calcium. I then close the lid *f'* and pass a current of electricity through the 50 contents. Under the influence of the heat caused by the resistance of the carbon a reaction sets in, which may be expressed by the following equation:



If sulfid of sodium is used instead of fluorid of sodium, the equation is as follows:



The fused mass of the alkali cyanid and calcium fluorid or calcium sulfid is drawn from the tap-hole *a'*, while the alkali metal volatilizes and passes through the pipe *g* into the 65 receptacle *h*. I then charge the furnace again and repeat the operation.

The mixture of cyanid and the other salt formed may be sold as such or the cyanid may be extracted from it by water and obtained in a pure state from such a solution by any known process.

I am well aware that it has been tried to convert an alkali nitrite by means of carbon in the free state into a cyanid, but I have 75 found that the output is very unsatisfactory, there taking place mainly reactions between oxygen and the carbon; but the large excess of alkali metal in my process *in statu nascendi* and the presence of carbon equally *in statu*. 80 *nascendi* prevent any such side reactions, the atmosphere within the furnace being a powerful reducing agent. At the same time I obtain the simultaneous production of two valuable substances, thus cheapening the 85 output of both.

What I claim is—

1. The process of simultaneously producing an alkali cyanid and an alkali metal, which consists in heating an alkali nitrite, another 90 alkali salt, and a carbid of an alkali-earth metal under exclusion of air, substantially as specified.

2. The process of simultaneously producing an alkali cyanid and an alkali metal, which 95 consists in heating an alkali nitrite in the presence of carbon *in statu nascendi* and in the presence of an alkali metal *in statu nascendi* under exclusion of air, substantially as specified.

Signed by me at Deadwood, South Dakota, this 4th day of June, 1903.

PAUL DANCKWARDT.

Witnesses:

R. N. OGDEN,  
G. E. FLAVIN.